

## UNITED STATES PATENT OFFICE

2,187,379

## ALLOY

Franz R. Hensel and Kenneth L. Emmert,  
Indianapolis, Ind., assignors to P. R. Mallory &  
Co., Inc., Indianapolis, Ind., a corporation of  
Delaware

No Drawing. Application June 2, 1939,  
Serial No. 276,993

5 Claims. (Cl. 75—173)

This invention relates to silver alloys of improved physical and electrical characteristics.

It is one of the objects of the invention to provide a silver base material which can be used for an electrical make and break contact, retaining very low contact resistance, having negligible material transfer and having great resistance to welding and sticking under severe electrical loads.

Another object of the invention is to provide a new silver base alloy which has increased tensile strength and which can be cold worked severely and retain a high annealing point, after such cold working.

It is a further object to provide a material which shows considerable improvements, as far as corrosion resistance is concerned.

Other objects of the invention will be apparent from the following description, taken in connection with the appended claims.

The present invention comprises a combination of elements, methods of manufacture, and the products thereof, brought out and exemplified in the disclosure hereinafter set forth, the scope of the invention being indicated in the appended claims.

While a preferred embodiment of the invention is described herein, it is contemplated that considerable variation may be made in the method of procedure and the combination of elements, without departing from the spirit of the invention.

The present invention contemplates an alloy of silver with magnesium and nickel. In the formation of the new alloy, it is preferable to provide a composition of the materials specified in the following proportions:

|           | Per cent                  |
|-----------|---------------------------|
| Magnesium | .05 to 15                 |
| Nickel    | 1 to 40                   |
| Silver    | Substantially the balance |

The preferred range of magnesium is .05 to 8%, because, up to that percentage, magnesium is taken up in alpha solution in silver and we have found that silver and magnesium up to 8% can be alloyed very readily, and the cast ingots can be rolled, swaged or drawn in the desirable shapes, such as sheet, bar stock, wire, strips or the like. The range of magnesium from 1 to 4% is especially useful.

Silver and nickel are mutually soluble only to a very limited extent, the solid solubility being only approximately 0.25% of nickel in silver. However, magnesium and nickel form alloys

with each other quite readily and by alloying magnesium with silver, it is possible to increase the solubility of nickel very materially and also hold excess nickel in suspension in the silver.

We have found it advisable if we use the larger percentage of nickel, however, to manufacture alloys, not by melting, but by sintering together the ingredients. By using the sintering method, which fundamentally consists in mixing the metal powders, pressing and sintering with or without additional re-sintering and re-pressing operations, we can incorporate nickel contents as high as 30 to 40%. Alloys of such high nickel content have the advantage that for applications such as electrical contacts, characteristics are obtained which provide a material that will not fuse together readily and that will show very small transfer.

If the alloys are to be used for chemical purposes, or other applications where a melted product is desired, the amount of nickel that is most desirable, ranges from about 0.25 to 5%. We have found in our studies that even with a small nickel content the annealing temperatures of cold worked material are raised by several hundred degrees Fahrenheit.

We have investigated a series of compositions, and we have found that the following ranges, which are given by way of example, have shown very excellent physical properties:

|               | Per cent   |
|---------------|------------|
| (1) Magnesium | 1 to 4     |
| Nickel        | .25 to 5   |
| Silver        | Balance 35 |
| (2) Magnesium | 2 to 8     |
| Nickel        | .25 to 5   |
| Silver        | Balance    |
| (3) Magnesium | 1 to 4     |
| Nickel        | 5 to 2.5   |
| Silver        | Balance 40 |
| (4) Magnesium | 1 to 8     |
| Nickel        | 15 to 40   |
| Silver        | Balance    |
| (5) Magnesium | 5 to 15    |
| Nickel        | 25 to 2.5  |
| Silver        | Balance    |
| (6) Magnesium | 5 to 15    |
| Nickel        | 2.5 to 30  |
| Silver        | Balance    |

The tensile strength of the improved alloys is materially increased by the combined addition of magnesium and nickel, without any appreciable loss of ductility. It is possible to obtain a Brinell hardness of 100 to 150° C., by proper

cold working. With a sufficiently high magnesium content, tensile strength values in the neighborhood of 50,000 pounds per square inch can even be obtained in the annealed condition.

- 5 The present alloy has outstanding merit if used for electrical purposes. In a comparison test, wherein contacts of similar dimensions were used on a resistive inductive circuit at 470 cycles per minute and wherein the current flowing in the 10 circuit was increased periodically, to obtain the definite current values of the alloys of the nature described above, in comparison with contact materials produced in the prior art, it was found that both the material transfer and the contact resistance 15 showed an improvement over the alloys of the prior art.

The alloys of the present invention have been found useful for a large number of electrical contact applications, such as for instance, sensitive 20 direct current relays, over-load cut outs, voltage regulators, indicating and recording gaugers, thermostatic controls and the like.

The other uses of the alloy are in the form of 25 silverware, particularly such silverware as is used for industrial applications, and where good corrosion resistance, high tensile strength and high annealing temperatures are required. Alloys may also be used for jewelry purposes and tableware.

30 Materials of the type described with a higher nickel content, can also be used for electrical brushes and arcing tips. It has been found advantageous to incorporate such materials as graphite into the mixture. It is also possible to

incorporate conductive oxides into the composition covered by the present invention. If, for certain applications, the material must retain a certain porosity, then a sintering process should be used which will provide a material with about 15 to 30% of voids. These voids can be later on filled with special oils or greases, in order to provide improved lubricating characteristics.

The alloy of the present invention has a commercial advantage, since the addition of magnesium in the percentage contemplated provides a material of lower specific gravity than the materials of the present art, and therefore it is possible to produce a larger number of finished products per unit weight of material. 10 15

While the present invention as to its objects and advantages has been described herein as carried out in specific embodiments thereof, it is not desired to be limited thereby, but it is intended to cover the invention broadly, within the 20 spirit and scope of the appended claims.

What is claimed is:

1. An alloy composed of .05 to 8% magnesium, .25 to 5% nickel, balance substantially all silver.
2. An alloy composed of 1 to 4% magnesium, .25 to 5% nickel, balance substantially all silver.
3. An alloy composed of 2 to 8% magnesium, .25 to 5% nickel, balance substantially all silver.
4. An alloy composed of 5 to 15% magnesium, .25 to 2.5% nickel, balance substantially all silver.
5. An alloy composed of .05 to 15% magnesium, .25 to 5% nickel, balance substantially all silver.

FRANZ R. HENSEL.

KENNETH L. EMMERT.